

## UNITED STATES PATENT OFFICE.

WILLIAM E. S. STRONG AND CHARLES E. PARSONS, OF NEW YORK, N. Y., AND SAMUEL PEACOCK, OF WHEELING, WEST VIRGINIA, ASSIGNORS TO METAL RESEARCH CORPORATION, OF NEW YORK, N. Y., A CORPORATION OF DELAWARE.

## PROCESS FOR MAKING METALLIC CHROMIUM.

No Drawing.

Application filed February 19, 1925. Serial No. 10,428.

*To all whom it may concern:*

Be it known that we, WILLIAM E. S. STRONG, a citizen of the United States, residing at New York, in the county of New York and State of New York, CHARLES E. PARSONS, a citizen of the United States, residing at New York, in the county of New York and State of New York, and SAMUEL PEACOCK, a citizen of the United States, residing at Wheeling, in the county of Ohio and State of West Virginia, have invented certain new and useful Improvements in Processes for Making Metallic Chromium; and we do hereby declare the following to be a full, clear, and exact description of the invention, such as will enable others skilled in the art to which it appertains to make and use the same.

This invention relates to a process for making metallic chromium in a shaft furnace of the type used in smelting ore, and has for its object to improve the procedures which have heretofore been proposed.

With this and other objects in view, the invention consists in the novel steps and combinations of steps constituting the process all as will be more fully hereinafter disclosed and particularly pointed out in the claims.

A modern iron ore smelting blast furnace with suitable equipment for blast heating, is capable of maintaining in its fusion zone a temperature of about 1600° C. in an atmosphere free from uncombined oxygen or carbon dioxide. According to this invention, the carbon in this zone of the furnace is maintained at a white heat, and under such conditions sodium oxide or salts containing sodium oxide, are brought into contact with such white hot carbon whereupon they are readily reduced to elemental sodium and carbon monoxide. The sodium thus produced is vaporized instantly upon its formation and rises with the gases of the furnace until it is cooled to about 750° C. by contact with the relatively cold charge in the upper part of said furnace, where said vaporized sodium condenses. But as it is molten above 100° C., said sodium continually moves downward by gravity in the form of a liquid and heats up again until it is again vaporized. By this means, a high concentration of sodium vapor is maintained at or near the 750° C. line of the

furnace, with an increase of its partial pressure. This effects an increase in the temperature necessary to vaporize the metal and a superheated state of the metal ensues.

Such heated liquid elemental sodium when in contact with chromium oxide will react as follows:—



This reaction with the reagents at about 800° C. has an exothermic thermal balance of about 836 B. t. u. per pound of chromium made. This is an energy gain capable of adding over 400° C. to the temperature reaction involved and thereby it increases the velocity of the reaction. Of course, the carbon present immediately reduces the sodium oxide produced back to elemental sodium.

It has been observed, however, that the somewhat impure metallic chromium thus produced takes the liquid form somewhat above the 1200° C. line of the furnace, and in falling through the charge material to the hearth, it contacts more or less with the white hot carbon in the fusion zone, and a small percentage of chromium carbide is formed. This carbide is decomposed by contact with the molten sodium present, but said molten sodium does not in any considerable mass extend much below the 1000° C. line of the furnace. It has been found that by introducing into the furnace through the tuyères sodium combined with oxygen, preferably in the form of sodium chromate, such chromium carbide as is formed is converted into sodium carbide and elemental chromium.

In the industrial operation of this process, an initial charge consisting of chromium oxide,  $\text{Cr}_2\text{O}_3$ , and an oxygen bearing sodium salt such as sodium carbonate and coke or charcoal is charged into the furnace in the usual manner of operating iron smelting blast furnaces and the metal is tapped from the hearth in the usual manner. Of course, chrome ores may be substituted for the above-mentioned chromic oxide. Although the slag formed is relatively small in quantity, yet, it is taken care of in the usual way. The sodium vapor reacts cyclically in the furnace however, as above intimated, and when a suitable equilibrium has been established, only such sodium is added to the furnace as is necessary to cover losses

due to slagging and losses at the throat of the furnace which are in the forms of carbides, cyanamids, etc. of sodium. If it is preferred to make good such losses, which amount approximately to 4% to 6%, the requisite amount of combined sodium is added through the tuyères.

The advantages of this process reside in the ability to make metallic chromium at 10 costs much less than in the procedures heretofore proposed and with an exceptional freedom from metalloid impurities.

What is claimed is:—

1. The process of making metallic chromium in a blast furnace, which consists in smelting a mixture containing chromic oxide, an oxygen bearing sodium compound and carbon causing the sodium to be liberated, volatilized and to react with the chromic oxide present to produce the desired metallic chromium.

2. The process of making metallic chromium in a blast furnace, which consists in

smelting a mixture containing chromic oxide an oxygen bearing sodium compound 28 and carbon causing the sodium to be liberated, volatilized and its partial pressure increased, and to react with the chromic oxide present to produce the desired metallic chromium.

3. The process of making metallic chromium in a blast furnace, which consists in smelting a mixture containing chromic oxide, an oxygen bearing sodium compound and carbon causing the sodium to be liberated, volatilized and to react with the chromic oxide present to produce sodium oxide and the desired metallic chromium and causing the carbon to reduce said sodium oxide back to elemental sodium.

In testimony whereof, we affix our signatures.

WILLIAM E. S. STRONG.  
CHARLES E. PARSONS.  
SAMUEL PEACOCK.